

No. 895,513.

PATENTED AUG. 11, 1908.

B. H. THWAITE & W. DEFRIES.  
MANUFACTURE OF MOLTEN METALS.

APPLICATION FILED AUG. 9, 1907.

3 SHEETS—SHEET 1.

Fig 1



Witnesses;

C. H. Fowler

P. A. Blair

## Inventors;

Benjamin H. Thwaite

Wolf Defries

By J. Walter Fowler  
their atty.

No. 895,513.

PATENTED AUG. 11, 1908.

B. H. THWAITE & W. DEFRIES.  
MANUFACTURE OF MOLTEN METALS.  
APPLICATION FILED AUG. 9, 1907.

3 SHEETS-SHEET 2.

Fig. 2



Fig. 3



Witnesses;  
C. J. Fowler  
R. H. Blair

Inventors;  
Benjamin H. Thwaite  
Wolf Defries  
By Walter Fowler  
their atty.

No. 895,513.

PATENTED AUG. 11, 1908.

B. H. THWAITE & W. DEFRIES.  
MANUFACTURE OF MOLTEN METALS.  
APPLICATION FILED AUG. 9, 1907.

3 SHEETS—SHEET 3.

Fig. 4



Fig. 6



Fig. 5



Fig. 7



Witnesses:  
G.W. Fowler

R. H. Blair

Inventors:  
Benjamin H. Thwaite  
f<sup>1</sup> Wolf Defries  
By J. Walter Fowler  
their atty

# UNITED STATES PATENT OFFICE.

BENJAMIN HOWARTH THWAITE AND WOLF DEFRIES, OF LONDON, ENGLAND.

## MANUFACTURE OF MOLTEN METALS.

No. 895,513.

Specification of Letters Patent. Patented Aug. 11, 1908.

Application filed August 9, 1907. Serial No. 387,776.

To all whom it may concern:

Be it known that we, BENJAMIN HOWARTH THWAITE, civil engineer, of 29 Great George street, Westminster, London, England, and WOLF DEFRIES, mechanical engineer, of 147 Houndsditch, London, England, have invented a certain new and useful Improvement in the Manufacture of Molten Metals, of which the following is a full, clear, and exact description, and for which we have applied for Letters Patent in Great Britain, No. 28,573, dated December 14, 1906.

The purpose of this invention is to obtain a more complete control over the composition of certain molten metals, such for example as steel, in the preparation of which large quantities of air or gas may be forced under pressure through the molten metal, and to shorten the process of manufacture which has been necessary hitherto for obtaining and refining a homogeneous product.

It consists substantially in a process of and means for using the blast to determine in the molten metal a systematic circulation during the continuance of which appropriate special treatment may be applied at a definite point or definite points in the vessel containing the metal, past which point or points fresh portions of the metal are continually brought.

The characteristic feature of the present invention is the employment of pneumatic means with mechanical structure to produce a continuous circulation of metal both to and from the surface and in and out of separate chambers, which chambers are wholly within the space occupied by the metal and wholly below its surface. In this manner we obtain a more rapid and complete mixture of the substances out of which the metal is manufactured, and the special treatment, if any, is applied directly to a much larger proportion of the metallic mass than in existing processes, so that a homogeneous product of desired composition is obtained more quickly and with greater certainty than is usually practicable.

A construction and operation embodying this process would be as follows, the description referring to the accompanying drawings in which:—

Figure 1 is a sectional elevation of an improved apparatus constructed in accordance with the invention, on line 1—1 of Fig. 2. Fig. 2 is a similar view on line 2—2 of Fig. 1. Fig. 3 is a cross section of the hollow trun-

nion on line 3—3 of Fig. 2. Figs. 4 to 7, are views in sectional elevation but on a smaller scale of modified shapes of the apparatus illustrated in Fig. 1.

The metallic mass intended for treatment is run into a vessel A composed, Fig. 1, of two vertical tubular limbs a, b communicating with each other through a continuous passage c in the lower part of the vessel and having an air space d closed at top and bottom between the inner faces of the vertical limbs a, b, extending from the top of the level of communication to the underside of the upper level above which the tubes coalesce to form a common chamber e. The external part of this vessel is made preferably in three or more portions united by flange rings A<sup>1</sup> the upper and lower portions being preferably split vertically as at flange joint A<sup>2</sup> for convenience of lining. The upper part e<sup>1</sup> is contracted into a throat e<sup>2</sup> somewhat of the form of that of an ordinary Bessemer converter.

The vessel A is lined with suitable refractory material B. The metal is filled to such a height as to overflow the top of the tubular limbs a, b, into the chamber e forming the upper part of the vessel which connects the tubular limbs, so as to provide a continuous volume of liquid metal above which the slag floats. At a suitable point in the lower part of the vessel, twyers f are arranged through which air delivered under pressure by pipes k, k<sup>1</sup> can be forced up one of the two vertical limbs. By employing a suitable pressure of air in our apparatus the introduction of such air determines a vigorous circulation of the molten metal, which flows up one limb a of the vessel and down the other limb b. One or more supplementary twyers f<sup>1</sup>, to which air is led through a branch pipe, k<sup>2</sup>, may be arranged in the upper part of the vessel to assist the downward flow through the limb b. If the metal in its downward circulation carries with it the slag or some proportion of it, that proportion will in this way be mixed more intimately with the mass of the metal than if it lay merely on the surface; and it will finally settle out when the vessel is tilted and the circulation is consequently finished.

The shape of the vessel is not limited to the precise form above described; we may for instance, bend one limb round on itself and arrange it so as to reenter at a point below the free surface, the blast being introduced

at or about the base of the shorter limb as shown in Fig. 4. Alternatively we may divide the vessel, which in such case might be, for example, egg-shaped, by a vertical diaphragm  $d^1$  of suitable refractory material right across the vessel, and open or furnished with passages at bottom, and stopping short of or perforated at the top, so as to permit the vigorous circulation of the metal when a blast is sent up one of the two chambers into which the vessel is divided: such arrangement is shown in Fig. 5. Alternatively we may as shown in Fig. 6 make the diaphragm last mentioned of an annular form, such as a hollow cylinder or cone  $d^2$ , wholly or partly open at bottom, at or about the base of which we let in the twyer blast vertically upwards. A contraction may if desired be formed opposite the tuyers  $f$  or at other suitable point or points by forming an enlargement or enlargements on the cone or its lining, or some portion of lining in the neighborhood of the twyer may be shaped so as to inclose the blast as it leaves the twyer mouth and act as a circulating ejector.

When it is desired to apply this system to an existing converter otherwise than by the means hereinbefore described, an external vertical tube  $b$  lined with refractory material 30 may be connected, see Fig. 7, to the converter at two points at different levels below the surface of the liquid, at the lower of which a twyer  $f^1$  is provided delivering a horizontal blast to force metal over the ordinary twyer 35 or tuyers  $f$  delivering a vertical blast from the center of the bottom of the vessel, and so connecting the metal in the vessel  $A$  and the external tube  $b$  by a continuous circulation. The essential part of the arrangements, 40 whether in respect of the shape of the apparatus or the nature and direction of the blast is in fact that it should be such that a definite circulation through the length of a continuous passage in the lower part of the vessel 45 should be established in the molten liquid so as to convey the metal continuously to and from its surface in the manner common to each of the examples which we have given.

In order to utilize the products of this process for assisting to maintain the temperature of the charge, when they are combustible and would ordinarily be consumed outside the vessel, a branch may be taken off the air supply by means of flexible metallic tubes 55 furnished with suitable valves or otherwise, and air may be led through it and delivered above the surface of the metal, so as to burn within the vessel any carbon monoxide, or other combustible gas that may be given off. 60 The air supply may be provided in the usual manner; but when the duration of the blowing process and the number of vessels are not sufficiently large to keep the blowing constant during the day, the air may be 65 derived from a motor and compressor de-

livering under relatively high pressure into an air reservoir or accumulator, from which it is drawn off through a suitable reducing valve as and when required. If the energy for this motor is derived from gas, a portion of 70 the generator gas from such a plant may be used for heating the interior of the vessel before introducing the molten metal.

The vessel is preferably arranged on trunnions  $g$  attached to a steel girdle  $h$  about its center, so as to allow it to be tilted by any usual contrivance for the purpose of pouring. The girdle  $h$  is clamped between cheek plates  $h^1$  which are bolted to collars  $h^2$  keyed on the axle  $g$ . In the form first above described, 75 see Figs. 1 and 2 the trunnions may afford a continuous axis, passing between the two vertical limbs  $a$   $b$ , and it may be hollowed in part as at  $g^1$  and provided with suitable ports  $g^2$  to serve for the introduction of air through 80 the pipe  $k$ , Fig. 3, upon the vessel being rotated through a given angle from the horizontal in the usual way. The vessel is shown journaled at  $l$  on pedestals  $m$  and its axle  $g$  is fitted with a worm wheel or segment  $n$  which 85 may be rotated by means of a worm in the well known manner.

Apart from the uses hereinbefore described, the following will illustrate the uses which may be made of the systematic circulation of 90 the metal past a given point or given points. If it be desired to introduce purifying or alloying substances they may be introduced on to the surface of the molten metal in the usual way or through a separate aperture in the 95 upper part of the vessel, or they may be introduced by obvious means with the blast itself. If it be desired to reduce the metal, a reducing gas may be introduced instead of or in succession to the blast, either through the 100 same or alternative tuyers of which the pneumatic operation is similar to that of the air tuyers. If it is not convenient to introduce such reducing gases under substantial pressure, they may be applied immediately 105 after the air blast has been shut off and before the circulation of the metal has stopped. If there is not sufficient heat within the mass of the metal to maintain it fluid, or if for any other reason it may be desirable, the reducing 110 gas may consist of or be accompanied by carbon or other suitable compounds of which the heat of combustion may compensate sufficiently for the heat lost in the reduction. If it be desired that the metal should have an increased proportion of carbon or any element which would be separated from a gas or vapor under the conditions in question, a 115 suitable gas or vapor may be introduced in a suitable manner.

For the convenience of foundry use, the vessel may be mounted on a wheeled or portable frame, and either connected with the blast by flexible tube or joined up with a high-pressure air main running round the foundry. 120 125 130

Having thus described our invention what we claim as such and desire to secure by Letters Patent is:—

1. The combination of a vessel adapted to contain a charge of molten metal, and means for introducing a blast below the level of the metal to maintain the molten metal in continuous circulation to and from the surface, said vessel having its interior fashioned with a continuous passage having separate ways for the respective movements of the molten mass.
2. The combination with a vessel adapted to contain a charge of molten metal, said vessel having a continuous passage with separate ways for the respective movements of the molten metal, and means for introducing first and second blasts into the separate ways of the vessel, said blasts respectively acting in the upward and downward directions so as to cause the metal to circulate definitely and continuously to and from the surface.
3. The combination with a vessel adapted to contain a molten metal, said vessel having a limb for ascending metal and a second limb for descending metal, and means disposed below the surface of the molten metal for causing the systematic and continuous circulation of the metal up and down the respective limbs to and from the surface of the molten metal.
4. The combination with a vessel adapted to contain molten metal, said vessel having a limb for ascending metal and a second limb for descending metal, said limbs connecting to form a continuous passage, twyers for introducing a blast into each of said passages below the surface of the metal, and in opposite directions, one of said blasts causing the metal to flow up and the other down the respective limbs to and from the surface of the molten metal.
5. For use in the manufacture of molten metals, a rotatable vessel lined with refractory material and comprising similar ascending and descending limbs, said vessel having a blast pipe introduced at the base of one of said limbs for the purpose of circulating the metal continuously to and from the surface.
6. For use in the manufacture of molten metals, a rotatable vessel lined with refractory material and comprising ascending and descending limbs, a blast pipe delivering along one of said limbs and a second blast pipe delivering along the other of said limbs in a direction opposite to the first, said blasts serving to circulate the metal continuously to and from the surface.

7. For use in the manufacture of molten metals, a rotatable vessel lined with refractory material and comprising ascending and descending limbs, a blast pipe delivering along one of said limbs and a second blast pipe delivering along the other of said limbs, said blasts serving to circulate the metal continuously to and from the surface and both being arranged to enter the vessel below the surface of the molten metal.

8. For use in the manufacture of molten metals, a vessel lined with refractory material and composed of two similar vertical tubular limbs said limbs communicating with each other through a continuous passage in the lower part of the vessel, a blast pipe introduced into the lower part of one of said limbs, said blast intended to circulate said molten metal continuously to and from the surface of the metal, and said vessel being mounted on bearings whereby it may be tilted in the manner of a Bessemer converter.

9. For use in the manufacture of molten metals, a vessel lined with refractory material and composed of two vertical tubular limbs, said limbs communicating with each other through a continuous passage in the lower part of the vessel, a blast pipe introduced into the lower part of one of said limbs, a second blast pipe introduced through the vessel and acting in direction opposite to the first, said blasts intended to circulate said molten metal continuously to and from the surface of the metal, and said vessel being mounted on bearings whereby it may be tilted in the manner of a Bessemer converter.

10. For use in the manufacture of molten metals, a vessel lined with refractory material and composed of two similar vertical tubular limbs, said limbs communicating with each other through a continuous passage in the lower part of the vessel, a blast pipe introduced into the lower part of one of said limbs, said blast intended to circulate said molten metal continuously to and from the surface of the metal, said vessel being made in a number of portions united by flange rings and having an upper part contracted into a throat, an axle on which said vessel is mounted and operating means whereby said vessel may be partly rotated.

In witness whereof we have hereunto set our hands in presence of two witnesses.

BENJAMIN HOWARTH THWAITE.  
WOLF DEFRIES.

Witnesses:

GEO. J. B. FRANKLIN,  
T. J. OSMAN.